

H. V. SEALE AND W. SHELLSHEAR,  
CONCENTRATION OF ORES,  
APPLICATION FILED JUNE 30, 1915.

1,311,919.

Patented Aug. 5, 1919.



H. V. Seale.  
W. Shellshear.  
Inventors.  
By *Sheridan & Smith*  
Attorneys.

# UNITED STATES PATENT OFFICE.

HARRY VERNON SEALE AND WILTON SHELLSHEAR, OF BROKEN HILL, NEW SOUTH WALES, AUSTRALIA, ASSIGNEES, BY MESNE ASSIGNMENTS, TO MINERALS SEPARATION NORTH AMERICAN CORPORATION.

## CONCENTRATION OF ORES.

1,311,919.

Specification of Letters Patent. Patented Aug. 5, 1919.

Application filed June 30, 1915. Serial No. 37,350.

To all whom it may concern:

Be it known that we, HARRY VERNON SEALE, by occupation mill superintendent, and WILTON SHELLSHEAR, by occupation metallurgist, subjects of the King of Great Britain, residing at Junction North Mine, Broken Hill, in the State of New South Wales, Commonwealth of Australia, have invented certain new and useful Improvements in the Concentration of Ores, of which the following is a specification.

This invention relates to certain improvements in the concentration of sulfid and other ores by what is commonly known as flotation separation. This invention is especially applicable to froth flotation separation in which the ores are subjected to aeration in an aqueous separating medium in the presence of a frothing agent for the formation of a froth or scum of the metalliferous mineral particles as is described, for example, in the United States Letters Patent No. 835120 of November 6, 1906; No. 962,678 of June 28, 1910; and No. 25 1,064,723 of June 17, 1913.

This invention is equally applicable to collective separation in which an indiscriminate float concentrate of metalliferous minerals is obtained as well as to differential or preferential flotation separation in which a float concentrate of certain metalliferous minerals from other metalliferous minerals is obtained.

This invention is applicable to the treatment of ores, concentrates, tailings, slimes or other metallurgical products and it will be understood that in this specification the term "ores" will include all such metallurgical products as well as crude materials.

40 Simplicity, economy, efficiency and reliability of construction and operation are the objects of the invention.

According to the present invention in the concentration of ores by flotation-separation, the ore pulp is fed by gravity with inclosure thereof in suitable conduits, and at intervals in the gravity flow of the ore, irruption of air to the inclosed pulp, and atomization or emulsification of the air, are caused so as to effect that degree of agitation and aeration of the pulp necessary for froth flotation. At other intervals in the flow of the pulp a condition of relative quiescence is produced such as will permit

the removal of froth by flotation, and the 55 froth is removed at these places of relative quiescence. Also according to the present invention a gravity flow of the pulp is produced with sufficient violence to induce irruption and atomization of air and the 60 froth is removed at successive points in the course of the gravity flow and the operation is regulated by adding liquid to the pulp at successive points in the flow of the pulp.

65 The expressions "air" and "aeration" are used in the following claims as understood in the art and are intended to include other suitable gases and gasification, as indeed air is but a mixture of gases in somewhat varying proportions.

70 Apparatus embodying the invention comprises a plurality of separating vessels and closed conduits arranged to convey the pulp by gravity through the separating vessels 75 successively and air-injecting means interposed in the conduits and operable by the gravity flow of pulp therein to inject air into the pulp. Such apparatus may comprise also a baffle arrangement for insuring 80 the proper emulsification or atomization of the air for the froth flotation process.

85 In order that the invention may be better understood we will now proceed to describe the invention with reference to the accompanying sheet of drawings in which

Figure 1 shows the arrangement of plant comprising a number of separating vessels in series.

Fig. 2 is a vertical section of one separating vessel and feed device therefor.

Fig. 3 shows a modified arrangement for effecting the purposes of this invention.

90 Each separating unit preferably comprises a separating box A and a feed box B. 95 The separating boxes A may be made of any convenient shape but we have found in practice that a cylindrical shape well answers the purpose. These feed boxes B are open at the top and are also of any 100 convenient shape but we have found that square shape in cross section well answers the purpose. Each feed box B is furnished with a depending feed pipe B' which delivers into the separating box A below the 105 level of the pulp or separating medium therein. The feed pipe B' delivers onto a baffle A' arranged within the separating

box A. Each separating box A is provided with launder A<sup>2</sup> for the float concentrates and a circular baffle A<sup>3</sup> surrounding the feed pipe B' for the purpose of maintaining a state of quiescence on the surface of the pulp in the separating vessel A. The vessel A is also furnished with an outflow A<sup>4</sup> for the unfloated residues which is provided with a removable annular plug or ring whereby the size of the same may be regulated. Leading from the outflow A<sup>4</sup> is a pipe or duct C which discharges into the next feed box B of the series. A main water pipe D is provided having taps or faucets D' adapted to discharge into the feed boxes B whereby the level therein may be adjusted and compensation made for losses occasioned by the withdrawal of concentrates. A common feed box or vessel E may be provided at the head of the series for the purpose of equalizing the feed so as to insure a regular flow to the apparatus.

In operation the pulp is fed from the equalizing feed box E into the first open feed box B whence it flows by the feed pipe B' into the first separating box or vessel A being delivered under the surface of the liquid striking the baffle A'. The float concentrates rise and overflow into the launder A<sup>2</sup> while the unfloated residues flow out through the hollow plug A<sup>4</sup> and the pipe or duct C to the next feed box B in the series and so on. The feed boxes B are open at the top and the flow of material thereto by the pipe C causes a vigorous agitation. The outflow through the pipes or tubes B' from the feed box B has a slight excess capacity over the flow of material therethrough so that a vortex or swirling action is set up which entraps air within the said pipes or tubes B' by the flow of material itself thereby insuring the requisite aeration necessary for the thorough emulsification of the pulp to effect flotation. The head or height of the feed box B above the separating box A is such as to regulate the flow of material to insure the aforesaid entrapping of air. The pulp with its entrapped air discharges immediately onto the baffle plate A' by which thorough emulsification is insured.

The outflow through the hollow plugs A<sup>4</sup> is controlled and regulated by adjusting the size thereof so that by having a series of hollow plugs A<sup>4</sup> of definite constant size the whole of the plant is self regulating providing the equalizing feed box E at the top is kept at a constant level or other means adopted for maintaining a constant feed. Water or aqueous separating medium is added to the various feed boxes B by the taps or faucets D' to compensate for that removed with the float concentrates and maintain a constant level with-

in the separating boxes A. This may also be effected by varying the size of the outflow orifices in the hollow plugs A<sup>4</sup>.

In practice the relative sizes or dimensions of the various parts of the apparatus will be regulated and adjusted as may be required to effect the purposes of this invention. We wish it to be understood that we do not confine ourselves to any precise sizes and dimensions but by way of illustration we may mention that we have successfully treated Broken Hill zinc-lead sulfid ores crushed to pass through a 40 mesh sieve and feeding at the rate of 20 tons per hour in a plant as illustrated in Figs. 1 and 2 of the accompanying drawings with the separating boxes A fifteen inches in diameter and twenty-four inches deep and the rest of the plant of proportional dimensions approximately as shown.

In the plant illustrated in Figs. 1 and 2 the feed boxes B are open at the top to allow of the entrapping of the air within the feed pipes B' by the flow of material itself. Other means may be provided for allowing of an inlet of air into the said feed pipe or tube B'. For example in the construction illustrated in Fig. 3 the feed pipe is provided with air inlets B<sup>2</sup> through which air may be drawn in for the aeration of the pulp. In this case the feed boxes may be dispensed with and the separating boxes A connected direct from one to the other by the pipe B' in sequence with sufficient height or head to insure the necessary flow of material.

The inventive idea and process embodied in the foregoing specific apparatus may be embodied and applied in other specific forms of apparatus by the exercise of the technical skill of the art, and still other adaptations may be inventively devised, all within the scope of the following claims.

We claim:

1. The process of concentrating ores which consists in producing a gravity flow of ore pulp with portions moving at high velocity and other portions in a state of relative quiescence, in the presence of a mineral frothing agent, and dropping the pulp in portions moving at high velocity into portions in a state of relative quiescence and below the liquid levels of said relatively quiescent portions, with inclosure of the pulp at its points of entrance into said relatively quiescent portions, and thereby carrying air into said relatively quiescent portions with such hydraulic violence of pulp flow as to subdivide the entrained air and agitate and aerate the pulp in that degree necessary for froth flotation, and removing the froth by flotation from such relatively quiescent portions of the pulp.

2. The process of concentrating ores which consists in producing a violent gravity flow

of ore pulp into a relatively quiescent body of pulp in the presence of a mineral frothing agent, by dropping the pulp into said relatively quiescent body and below the liquid level of said relatively quiescent body, with inclosure of the pulp at its point of entrance into said relatively quiescent body, and thereby carrying air into said relatively quiescent body with such hydraulic violence of pulp flow as to subdivide the entrained air and agitate and aerate the pulp in that degree necessary for mineral-froth-flotation, and removing the mineral froth by flotation from the surface of such relatively quiescent body of pulp.

3. The process of concentrating ores which consists in producing a violent gravity flow of ore pulp into a relatively quiescent body of pulp in the presence of a mineral-frothing agent, by dropping the pulp into said quiescent body, with inclosure of the dropping pulp, except for access of air at the upper portion of the dropping pulp, the inclosure being continued to a point below the liquid level of the relatively quiescent body, so as to carry air with the dropping pulp below the surface of said relatively quiescent body and thereby cause irruption of air in the quiescent body of pulp and effect therein that degree of agitation and aeration necessary for froth flotation and the formation of a mineral-bearing froth at the surface of the quiescent pulp body, and separating such froth.

35 4. The process of concentrating ores which consists in producing a gravity flow of ore pulp containing a mineral-frothing agent, with rapid movement in portions of such flow and relative quiescence at other portions of such flow, and delivering the rapidly moving portions of the pulp to the relatively quiescent bodies of the pulp by dropping the pulp with inclosure thereof except for access of air at upper portions of such dropping pulp, the inclosure being continued to points below the liquid levels of the relatively quiescent bodies of such pulp, so as to carry air with the pulp below the surface of such relatively quiescent bodies of pulp and thereby to cause irruption of air in such quiescent bodies of pulp and effect that degree of agitation and aeration of the pulp necessary for mineral-froth-flotation and the formation of mineral-bearing froth at the surfaces of such quiescent bodies of pulp, and separating such froth.

5. The process of concentrating ores by froth-flotation which consists in producing a gravity flow of ore pulp containing a mineral-frothing agent with sufficient violence to induce irruption and subdivision of air and aeration of the pulp in that degree necessary to form a mineral-bearing froth, and removing the resultant froth by flotation at successive points in the course of said

gravity flow of the pulp, and adding liquid to the pulp at successive points in its flow in a measure to compensate for the liquor removed with the froth and to regulate the pulp flow.

6. The process of concentrating ores by froth-flotation which consists in producing a gravity flow of ore pulp containing a mineral-frothing agent with sufficient violence to induce irruption and subdivision of air and aeration of the pulp in that degree necessary to form a mineral-bearing froth, producing relative quiescence of the pulp at successive points in the course of said gravity flow, removing the froth by flotation at such quiescent places, and adding liquid to the pulp at successive points in its flow in a measure to compensate for the liquor removed with the froth and to regulate the pulp flow.

7. Apparatus for the concentration of ores by froth flotation comprising a number of separating vessels at successive levels, and closed conduits including air-injecting means operable by pulp flow to entrain air into the conduits with the pulp, said conduits being arranged to convey the pulp by gravity through said separating vessels successively and to deliver the pulp flow to each vessel below the liquid level therein with hydraulic violence resulting from gravity sufficient to subdivide said entrained air and aerate and agitate the pulp below said liquid level in each separating vessel in that degree necessary to form a mineral-bearing flotation froth.

8. Apparatus for the concentration of ores by froth flotation comprising a number of separating vessels at successive levels, closed conduits including air-injecting means operable by pulp flow to entrain air into the conduits with the pulp, said conduits being arranged to convey the pulp by gravity through said separating vessels successively and to deliver the pulp flow to each vessel below the liquid level therein with hydraulic violence resulting from gravity sufficient to subdivide said entrained air and aerate and agitate the pulp below said liquid level in each separating vessel in that degree necessary to form a mineral-bearing flotation froth, and a quieting baffle in each separating vessel disposed between the point of pulp delivery thereto and the liquid level therein.

9. Apparatus for the concentration of ores by froth flotation comprising a number of separating vessels at successive levels, agitation baffles in said vessels below their liquid levels, and closed conduits including air-injecting means operable by pulp flow to entrain air into the conduits with the pulp, said conduits being arranged to convey the pulp by gravity through said separating vessels successively and deliver the pulp flow

70

75

85

90

95

100

105

110

115

120

125

130

- to each vessel below its liquid level and against its agitation baffle with hydraulic violence resulting from gravity sufficient to subdivide said entrained air and aerate and 5 agitate the pulp below said liquid level in each separating vessel in that degree necessary to form a mineral-bearing flotation froth, the agitation baffles being located in the path of the rapidly falling pulp.
10. Apparatus for the concentration of ores by froth flotation comprising a number of separating vessels at successive levels, agitation baffles in said vessels below their liquid levels, closed conduits including air-injecting means operable by pulp flow to entrain air into the conduits with the pulp, said conduits being arranged to convey the pulp by gravity through said separating vessels successively and deliver the pulp flow to 15 each vessel below its liquid level and against its agitation baffle with hydraulic violence resulting from gravity sufficient to subdivide said entrained air and aerate and agitate the pulp below said liquid level in each 20 separating vessel in that degree necessary to form a mineral-bearing flotation froth, and a quieting baffle in each separating vessel disposed between its liquid level and the point of pulp delivery against its agitation 25 baffle.
11. Apparatus for the concentration of ores by froth flotation comprising a separating vessel, an agitation baffle therein below its liquid level, a source of ore pulp, and 30 a closed conduit including air-injecting means operable by pulp flow to entrain air into the conduit with the pulp, said conduit being arranged to convey the pulp by gravity from said source and deliver it to the 35 separating vessel below its liquid level and against its agitation baffle with hydraulic violence resulting from gravity sufficient to subdivide said entrained air and aerate and agitate the pulp below said liquid level in the 40 separating vessel in that degree necessary to form a mineral-bearing flotation froth.
12. Apparatus for the concentration of ores by flotation-separation comprising a 45 separating vessel having a residues outflow at the bottom, a feed box open at the top and having an inflow pipe at the side thereof and a discharge pipe at the bottom forming a pulp-operated air injector and of such length as to deliver air and pulp at high 50 velocity produced by gravity flow therein into the said separating vessel below the surface of the liquid therein.
13. Apparatus for the concentration of 55 ores by flotation-separation comprising a separating vessel having a residues outflow at the bottom a feed box open at the top and having a discharge pipe at the bottom form-

ing a pulp-operated air injector and of such length as to deliver air and pulp at high 65 velocity produced by gravity flow therein into the said separating vessel below the surface of the liquid therein, and a baffle arranged within the said separating vessel in the path of the inflowing air and pulp.

14. Apparatus for the concentration of ores by flotation-separation comprising a separating vessel having a regulatable residues outflow at the bottom, and a feed box open at the top and having a discharge pipe 75 at the bottom forming a pulp-operated air injector and of such length as to deliver air and pulp at high velocity produced by gravity flow therein into the said separating vessel below the surface of the liquid 80 therein.

15. Apparatus for the concentration of ores by flotation-separation comprising a separating vessel having a regulatable residues outflow at the bottom, a feed box open 85 at the top and having a discharge pipe at the bottom forming a pulp-operated air injector and of such length as to deliver air and pulp at high velocity produced by gravity flow therein into the said separating 90 vessel below the surface of the liquid therein, and an agitating baffle arranged within the said separating vessel in the path of the inflowing air and pulp.

16. Apparatus for the concentration of 95 ores by flotation-separation comprising a separating vessel having a float concentrates launder at the top and a regulatable residues outflow at the bottom, a feed box open at the top and having an inflow pipe 100 at the side thereof and a discharge pipe at the bottom forming a pulp-operated air injector and of such length as to deliver air and pulp at high velocity produced by gravity flow therein into the said separating 105 vessel below the surface of the liquid therein, and an agitating baffle arranged within the said separating vessel in the path of the inflowing air and pulp.

17. In combination, a plurality of separating receptacles each having pulp delivery means adapted to inject air into the pulp by the flow of the pulp, the discharge means of the higher of the series being connected to the feed means of the lower, and provided with regulating means adapted to control the volume of pulp discharge and thereby the injection of air into said pulp.

In testimony whereof we affix our signatures in presence of two witnesses.

HARRY VERNON SEALE.  
WILTON SHELLSHEAR.

Witnesses:

ANTHONY HALL,  
STEPHEN EDGAR WELLINGTON.